

Dec. 29, 1953

C. CITO

2,663,921

METHOD FOR THE CENTRIFUGAL CASTING OF METAL PARTS

Filed June 8, 1949



Inventor  
By, Camillo cito.

  
Attorneys.

## UNITED STATES PATENT OFFICE

2,663,921

METHOD FOR THE CENTRIFUGAL  
CASTING OF METAL PARTS

Camillo Cito, Uccle, Belgium, assignor to Industrial Research Laboratory Inc., Philadelphia, Pa.

Application June 8, 1949, Serial No. 97,788

2 Claims. (Cl. 22—200.5)

1

The present invention relates to a method for the centrifugal casting of metal parts of annular shape in a rotary mould.

The structural claims originally embodied in this application have been divided and are included in divisional application Serial No. 153,365, now abandoned, filed April 1, 1950, for Installation for the Centrifugal Casting of a Metal Ingot of General Annular Shape.

The annular castings hitherto obtained by this method had cracks or other faults on the cylindrical periphery, which must be attributed to the high co-efficient of heat transmission of the walls of the cylindrical mould, and also frequently, lacked homogeneity, which was essentially due to irregularities in the temperatures of casting and cooling heretofore used.

The present invention has for its object to obtain by centrifugal casting annular metal parts of homogeneous structure, without cracks, fissures or any solid and/or gaseous inclusions.

According to the invention, the centrifugal casting of the annular part is effected under thermal conditions that prevent a substantial accumulation of heat in the walls of the mould, and which are such that the solidification by cooling on said walls, from the outside towards the inside, can be varied, on the one hand in relation to the mass of metal being treated, and on the other hand in relation to the speed of rotation used in the centrifugal casting operation, it being possible for said speed and said cooling also to be varied at every instant in relation to the increase in the mass being cast during the process of casting and forming the said part.

This centrifugal casting according to the invention can be effected about a horizontal axis and the said thermal conditions can be obtained by means that comprise an internal or axial heating and an external cooling of the mass, which is dependent from the speed of rotation of the mass being treated, which determines its centrifugal force, and from an adjustable stream of cooling air applied to the external periphery of a cylindrical mould, the walls of which have only a slight calorific inertia, so that it is possible to reduce and/or adjust at will the loss of heat of said mould.

The invention thus provides in the first place, conditions that enable the temperature of the external peripheral surface of the ingot in contact with the walls of the mould to be adjusted by slowing down the losses of heat, thereby preventing the formation of cracks on the said peripheral surface of the ingot. It also enables a uniform distribution of the molten metal in the

2

rotary mould to be obtained at every instant, and also enables the regularity of settling of the mass being treated to be obtained by keeping the force of cohesion predominant by the action of adjustable speeds of rotation, with the methodical elimination of inclusions and gases, by the adjustment of the cooling, starting from the periphery towards the centre of the cylindrical ingot in course of formation.

10 Other features and details of the invention will become apparent from the following description made with reference to the drawings which are annexed to the present specification and which show an equipment intended for the manufacture of annular ingots with a cylindrical periphery.

In these drawings:

Fig. 1 shows an elevational view of the equipment with portions broken away, and

Fig. 2 is a section through the vertical plane II—II of Fig. 1, showing also the means for cooling and rotating the rotary mould, and also the casting operation.

The equipment shown comprises a cylindrical mould 2 which is adapted to be rotated about a horizontal axis I—I. The mould is provided at both its ends with cheeks 3 and 4 which limit the width of the ingot and are engaged over a cylindrical drum or wall 5 which is of only comparatively small thickness. This cylindrical wall 5 is provided on the outside with fins 6 which are at right angles to the axis of rotation I—I and are arranged evenly and parallel to one another between the cheeks 3 and 4, which rest on four rollers 7 and 8 mounted respectively on shafts 9 and 10. The shaft 9 is the driven shaft of a speed variator 11 for the motor 12. If it be assumed that the shaft 9 rotates in the direction of the arrow X, the mould, therefore rotates in the direction of the arrow Y. A fan 13, the rotor of which is driven, for example, by means of a belt 14 running on a pulley 15 of the shaft 9, forces air through a pipe 16 on to the fins 6 in the direction of the arrow Z. The pipe 16 is therefore so located that the jet of air that issues therefrom is directed in the opposite direction to the direction of rotation of the mould 2.

A valve 17 is fitted on the delivery pipe 16 to enable the quantity of air blown on to the fins 6 to be adjusted even when the speed of rotation of the rollers remains unchanged.

The mould 2 is furthermore equipped with a source of heat in its central zone. The said source of heat is shown in the form of two carbon electrodes 18—19' between which an electric arc can be struck to heat the inside of the mould.

In order to cast, for example, a mild steel ingot

in the plant which has just been described, it is advantageous to proceed as follows:

To avoid direct contact of the metal to be cast with the thin cylindrical wall 5 of the mould, the inside of the mould may be coated with milk of silica and bentonite or it is possible to distribute the refractory layer 19 to be formed by centrifugal action and gradual heating. At the same time, the joints formed between the cylindrical wall 5 and the cheeks 3 and 4 have thus been filled, 10 whereby subsequent stripping is facilitated.

After having heated the inside of the mould 2 so as to raise it to a temperature of about 400° C., the casting operation is started, for example by quickly pouring into said mould from a crucible 20 a mass of steel in quantity sufficient for it not to solidify and subjecting it to centrifugal action. The steel is poured at a temperature that may advantageously be between 1,500° and 1,600° C. The steel is then poured 15 as slowly as possible, so that the layers of liquid which form are as thin as possible. This greatly facilitates the evenness of the settling and the elimination of the gases and impurities, while during the solidification of the ingot it is important to control the speed of rotation of the mould in order to obtain a satisfactory homogenization during cooling. This cooling does not only vary with the speed of rotation of the mould, but also depends on the position of the valve 17. The orientation of the delivery pipe 16 for the air in the opposite direction to the direction of 20 rotation of the fins 6 enhances the cooling, since the relative speed is equal to the sum of the linear speeds of the air stream and of said fins, so that the temperature of the mould may advantageously be maintained at a maximum value of about 550° to 600° C. In this manner, owing to the low calorific inertia of the mould and the possibility of adjusting the loss of heat, it is possible to keep said loss of heat at a low value during the casting operation and for some time after the completion of same, and this adjustment can also be used to increase said loss subsequently to such a degree that the temperature of the mould does not greatly exceed about 550° C.

It should be noted in particular that with this method of the invention, the value of the loss of heat in the mould, which can be varied at will, can be expressed by the formula:  $a=2+10\sqrt{v}$  wherein  $v$  is the relative peripheral speed of the air with respect to the rotating mould.

In the case, for example, of an annular mild steel ingot of about fifty kg. the casting in a mould of suitable size is effected as follows:

During a first phase that corresponds to the beginning of the casting operation, the heated mould is rotated at such an angular speed that the centrifugal force developed is at least twice that necessary for the molten metal to assume the shape of a ring in contact with the mould. The approximate peripheral speed  $V$  of the mould at this point may be expressed as  $V^2=2gr^2/r'$  where  $g$  is the acceleration of gravity,  $r$  is the radius of the inside of the mould and  $r'$  is the radius of the inside of the ingot. This first phase may be completed in about ten minutes, while the casting has been effected after about two minutes.

During a second phase, the supply of heat is cut down and the above-mentioned peripheral speed is reduced to a speed such that the centrifugal force is approximately that necessary to cause the fluid metal to take the form of a ring 75

in contact with the mould. The approximate peripheral speed  $V_1$  at this point is expressed as  $V_1^2=gr^2/r'$ . This second phase can be complete in about 15 minutes.

In a third phase, the peripheral speed is increased. It is at the beginning of this phase, as the metal cools to about 600-550° C., that the final settling of the cast metal starts, with the elimination of the last traces of gases. The centrifugal force that acts during this third and final phase, which may last one hour and a half, is therefore about three times that required for the molten metal to assume the shape of a ring in contact with the mould. The peripheral speed  $V_2$  at this point is expressed as  $V_2^2=3gr^2/r'$ .

When the centrifugal action has been stopped, one of the two side cheeks is removed. The annular ingot can then be readily removed owing to the contraction of the metal, and it is allowed to cool slowly for about forty-eight hours, covered with hot ashes.

When examined under the microscope, it was observed that the ingot had a totally different molecular structure from that of steel cast in the ordinary manner. Whereas the normal molecular structure of a well refined good cast steel is in the form of distinctly visible grains of ferrite surrounded by grains of pearlite, the steel which has been cast by the method according to the invention, on the contrary, shows under the microscope a structure almost similar to that of forged steel, without segregations of impurities and without blow-holes.

The invention is not restricted to the manufacture of ingots of annular shape with a cylindrical outer surface, but can also be applied to parts such as gears or the like, the outer periphery of which departs from the cylindrical shape. In this case, a rotary mould or drum 40 may be used, the inner contour of which corresponds to the shape of the desired part, without exceeding the scope of the following claims.

What I claim is:

1. The process of centrifugally casting a metallic ringlike ingot, using a metallic mould having a thin wall, which comprises rotating the thin walled metallic mould about its own axis in a horizontal position of the axis at an approximate minimum peripheral speed  $V$  expressed as  $V^2=2gr^2/r'$  where  $g$  is the acceleration of gravity,  $r$  is the radius of the inside of the mould and  $r'$  is the radius of the inside of the ingot, preheating the interior of the mould to a temperature of about 400° C., cooling the periphery of the mould be a stream of air directed on the outside of the mould, pouring molten metal into the preheated mould and forming the molten metal into a ring in contact with the inside of the mould, continuing the heating of the interior of the mould to heat the metal during the pouring and at least until the entirety of the molten metal cast has taken the ring form in the mould, subsequently stopping interior heating of the mould, subsequently reducing the approximate peripheral speed of the mould to a new value  $V_1$  expressed as  $V_1^2=gr^2/r'$  and for a time at least equal to that of the pouring operation, then increasing the approximate peripheral speed of the mould to a new value  $V_2$  expressed as

and further regulating the cooling rate so that the temperature of the mould does not exceed about 550° C.

2. The process of centrifugally casting a me-

tallic ringlike ingot, using a metallic mould having a thin wall, which comprises turning the thin walled metallic mould on its own axis in horizontal position of the axis at an approximate minimum peripheral speed  $V$  expressed as

$$V^2 = 2gr^2/r'$$

where  $g$  is the acceleration of gravity,  $r$  is the radius of the inside of the mould and  $r'$  is the radius of the inside of the ingot, preheating the interior of the mould to about  $400^\circ$  C., cooling the outside of the mould by a stream of air, pouring the molten metal into the preheated mould and forming the molten metal into a ring in contact with the inside of the mould, continuing the heating of the interior of the mould to heat the metal during the casting and at least until all the molten metal to be cast has taken the ring form on the inside of the mould, subsequently stopping the heating of the inside of the mould, reducing the approximate peripheral speed of the mould to a new value  $V_1$  expressed as  $V_1^2 = gr^2/r'$  and for a time of about one and one-half times the time which elapsed since the beginning of the pouring, then increasing the approximate peripheral speed of the mould to a new value  $V_2$  expressed as  $V_2^2 = 3gr^2/r'$  and regulating the cooling by regulating the air stream in a direc-

tion opposite to the direction of rotation in order to maintain the temperature in the mould not exceeding  $550^\circ$  C.

CAMILLO CITO.

References Cited in the file of this patent

UNITED STATES PATENTS

| Number    | Name          | Date          |
|-----------|---------------|---------------|
| 644,018   | Lilienberg    | Feb. 20, 1900 |
| 1,277,543 | Carney        | Sept. 3, 1918 |
| 1,349,416 | Eynon         | Aug. 10, 1920 |
| 1,436,305 | Cammen        | Nov. 21, 1922 |
| 1,573,089 | Rice          | Feb. 16, 1926 |
| 1,698,623 | Dale          | Jan. 8, 1929  |
| 1,698,624 | Dale          | Jan. 8, 1929  |
| 1,783,094 | Moore et al.  | Nov. 25, 1930 |
| 1,882,516 | Naugle et al. | Oct. 11, 1932 |
| 1,957,718 | Naugle et al. | May 8, 1934   |
| 1,993,774 | De Bats       | Mar. 12, 1935 |
| 2,087,347 | Larsen        | July 20, 1937 |
| 2,252,219 | Trotzke       | Aug. 12, 1941 |

FOREIGN PATENTS

| Number  | Country | Date          |
|---------|---------|---------------|
| 871,918 | France  | Jan. 22, 1942 |

OTHER REFERENCES

The Iron Age, page 81, May 26, 1949.